

## UNITED STATES PATENT OFFICE

2,207,554

CORROSION RESISTANT AND COLD WORK-  
ABLE MOLYBDENUM STEELHeinrich Reitz, Bitterfeld, and Erich Hengler and  
Alfred Bütinghaus, Wetzlar, GermanyNo Drawing. Application March 10, 1938, Se-  
rial No. 195,104. In Germany May 7, 1935

1 Claim. (Cl. 75—126)

The present application relates to steels capable of resisting attack by corrosive media including aqueous solutions of chlorine, hypochlorous acid and their salts and is a continuation-in-part of our co-pending application Serial No. 78,316 filed May 7, 1936.

One of the chief problems with which the present day metallurgists are faced is a meeting of the demand by the chemical arts for steels which 10 will withstand corrosive chemicals and still be capable of being mechanically worked. This problem is particularly onerous as regards those industries which employ solutions of chlorine-containing substances, since, as is known, ferrous metals are very susceptible to attack by these substances. In fact, screens and the like used 15 in filtering apparatus in the manufacture of hypochlorites, when made of so-called stainless steel, are so vigorously attacked that their utility is completely impaired after only short periods 20 of service.

Chromium is one of the alloying elements which is most commonly employed in steels designed for use in chemical apparatus. This element has the function, among others, of improving the corrosion resistance of the steel. Molybdenum has recently come into rather extended use, usually 25 with chromium as an agent for increasing or imparting corrosion resistance. Neither this element nor chromium, nor both together, however, is capable of giving steels this property to an extent sufficient to withstand the attack of different chemicals especially solutions of chlorine-containing substances. Moreover, molybdenum, 30 when used in large amounts, has a marked tendency to render steels brittle thereby impairing their capability of being mechanically worked in the cold, that is cold rolled, cold drawn and cold hammered. Any increase in corrosion resistance 35 resulting from the use of large proportions of molybdenum is, therefore, offset by a decrease in the mechanical cold workability of the steels.

The purpose of this invention is to provide a chromium-molybdenum low-carbon steel which 40 will be resistant to attack by aqueous solutions of chlorine, hypochlorous acid, their salts and the like, and at the same time will possess the desired mechanical properties of being cold rolled, cold drawn, cold hammered and the like to a high 45 degree.

We have discovered that if there is included in low carbon-chromium-molybdenum steels an alloying ingredient capable of forming carbides, in such quantities that after a fixing of the free carbon as carbide there remains sufficient of the 15 ingredient to form mixed crystals with the other alloying ingredients, steels of a resistance to chlorine-containing solutions which could not be foreseen are obtained. The alloying ingredient that we have found most suitable for use and which we therefore prefer, is titanium. Preferably the titanium is present in an amount from about 6 to 12 times the amount of the carbon present. However, other elements may be used in lieu of titanium with satisfactory results. Thus, 20 such carbide-forming elements as vanadium, tantalum, uranium, niobium, cerium, boron, zirconium and tungsten may be used as substitutes for titanium. It is of course to be understood that when such other carbide-forming elements are used to replace the titanium, they will 25 be used in amounts equivalent to the amount of titanium employed. In this connection cognizance should be taken of the fact that titanium carbide has the formula  $TiC$ ; vanadium carbide the formula  $VC$ ; tantalum carbide the formula  $TaC$ ; uranium carbide the formula  $U_2C_3$ ; niobium carbide the formula  $NbC$ ; cerium carbide the formula  $CeC_2$ ; boron carbide the formula  $B_6C$ ; zirconium carbide the formula  $ZrC_2$  and tungsten 30 carbide the formula  $W_2C$ . It will be seen from a simple computation based on these formulae and the molecular weights of the elements in question that for each part of titanium there should be used about 1.1 parts of vanadium; about 3.8 parts of tantalum; about 7.5 parts of uranium; about 1.9 parts of niobium; about 1.45 parts of cerium; about 1.4 parts of boron; about 1 part of zirconium and about 7.6 parts of tungsten.

As previously noted, we have found it preferable in making up our alloys to maintain a low content of carbon, that is less than about 5%. The chromium content of the alloys should range between about 12 and 30%, preferably between about 20 and 30%. The molybdenum content 45 may be as high as 5% and should exceed about 1.5%. The titanium should be present in an amount of from about .5 to 3.5%. The same is true if vanadium or zirconium is used in place of titanium. On the other hand, if boron or cerium 50

be so used, they will be present in an amount of from about .7 to about 5%. The amount of tantalum which would be employed in lieu of titanium would be about 1.9 to about 13.3%. The quantity 5 of uranium or tungsten which would be present as a substitute for the amount of titanium would be from about 3.8 to about 26.3%. Niobium, if used, would be present in an amount of from about .9 to about 6.7%. The addition of small amounts 10 of manganese and silicon are also to be recommended. Thus the steel preferably contains from about .3 to about .6% of manganese and less than .5% of silicon. The addition of copper in an amount not exceeding 3% has the effect 15 of further increasing the corrosion resistance of the steel. The balance of the steel is iron with the usual negligible quantities of impurities generally present in stainless steels.

These steels, especially when prepared with titanium, not only are remarkably resistant to corrosion by chlorine-containing solutions but also possess the property of being cold rolled, cold hammered and cold drawn. An estimate of their 20 resistance to corrosion may be gleaned from the fact that said steels are capable of withstanding attack by the very corrosive calcium hypochlorite solutions even at a temperature of 110° C. Said steels may, therefore, be employed for all purposes where steels of these properties are required. 25 Thus they are admirably fitted for the manufacture of wire screens for filtering chlorine- and hypochlorite-containing mashes and lyes and perforated supporting discs for such filters as well as armatures, armature accessories, pumps, 30 containers, valves, slide bars and the like which during use contact chlorine-containing solutions.

The following illustrates typical alloys within the scope of our invention:

|    |                                                             | Per cent         |
|----|-------------------------------------------------------------|------------------|
| 40 | (1) Carbon                                                  | = less than 0.50 |
|    | Manganese                                                   | = 0.30- 0.60     |
|    | Silicon                                                     | = less than 0.50 |
|    | Chromium                                                    | = 12.5-30.0      |
|    | Molybdenum                                                  | = 1.50- 5.00     |
| 45 | Titanium                                                    |                  |
|    | Vanadium                                                    | = .5 - 3.5       |
|    | or Zirconium                                                |                  |
|    | or                                                          |                  |
|    | Uranium                                                     |                  |
| 50 | or Tungsten                                                 | = 3.8 -26.3      |
|    | or                                                          |                  |
|    | Niobium                                                     | = .9 - 6.7       |
|    | or                                                          |                  |
|    | Cerium                                                      |                  |
| 55 | or Boron                                                    | = .7 - 4.25      |
|    | Balance iron and negligible quantities of usual impurities. |                  |
|    |                                                             | Per cent         |
| 60 | (2) Carbon                                                  | = less than 0.10 |
|    | Manganese                                                   | = 0.40- 0.60     |
|    | Silicon                                                     | = less than 0.50 |
|    | Chromium                                                    | = 16.0-18.0      |
|    | Molybdenum                                                  | = 1.80- 2.40     |
| 65 | Titanium                                                    | = 0.80- 1.20     |
|    | Balance iron and negligible quantities of usual impurities. |                  |
|    |                                                             | Per cent         |
| 70 | (3) Carbon                                                  | = 0.20- 0.30     |
|    | Manganese                                                   | = 0.40- 0.60     |
|    | Silicon                                                     | = less than 0.50 |
|    | Chromium                                                    | = 23.0-25.0      |
|    | Molybdenum                                                  | = 2.80- 3.30     |
|    | Titanium                                                    | = 1.80- 2.40     |
| 75 | Balance iron and negligible quantities of usual impurities. |                  |

|     |                                                                                                                                                                                                                                                                                                                                                                                                                                                                                                                                                                                                                                                                                                                                                               | Per cent         |    |
|-----|---------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|------------------|----|
| (4) | Carbon                                                                                                                                                                                                                                                                                                                                                                                                                                                                                                                                                                                                                                                                                                                                                        | = 0.18- 0.22     |    |
|     | Manganese                                                                                                                                                                                                                                                                                                                                                                                                                                                                                                                                                                                                                                                                                                                                                     | = 0.40- 0.60     |    |
|     | Silicon                                                                                                                                                                                                                                                                                                                                                                                                                                                                                                                                                                                                                                                                                                                                                       | = less than 0.50 |    |
|     | Chromium                                                                                                                                                                                                                                                                                                                                                                                                                                                                                                                                                                                                                                                                                                                                                      | = 27.0-29.0      | 5  |
|     | Molybdenum                                                                                                                                                                                                                                                                                                                                                                                                                                                                                                                                                                                                                                                                                                                                                    | = 1.60- 2.00     |    |
|     | Titanium                                                                                                                                                                                                                                                                                                                                                                                                                                                                                                                                                                                                                                                                                                                                                      | = 1.20- 1.60     |    |
|     | Balance iron and negligible quantities of usual impurities.                                                                                                                                                                                                                                                                                                                                                                                                                                                                                                                                                                                                                                                                                                   |                  |    |
| (5) | Carbon                                                                                                                                                                                                                                                                                                                                                                                                                                                                                                                                                                                                                                                                                                                                                        | = less than 0.50 | 10 |
|     | Manganese                                                                                                                                                                                                                                                                                                                                                                                                                                                                                                                                                                                                                                                                                                                                                     | = 0.40- 0.60     |    |
|     | Silicon                                                                                                                                                                                                                                                                                                                                                                                                                                                                                                                                                                                                                                                                                                                                                       | = less than 0.50 |    |
|     | Chromium                                                                                                                                                                                                                                                                                                                                                                                                                                                                                                                                                                                                                                                                                                                                                      | = 20.0-30.0      |    |
|     | Molybdenum                                                                                                                                                                                                                                                                                                                                                                                                                                                                                                                                                                                                                                                                                                                                                    | = 1.80- 4.00     | 15 |
|     | Titanium                                                                                                                                                                                                                                                                                                                                                                                                                                                                                                                                                                                                                                                                                                                                                      |                  |    |
|     | Vanadium                                                                                                                                                                                                                                                                                                                                                                                                                                                                                                                                                                                                                                                                                                                                                      | = .5 - 3.5       |    |
|     | or Zirconium                                                                                                                                                                                                                                                                                                                                                                                                                                                                                                                                                                                                                                                                                                                                                  |                  |    |
|     | or                                                                                                                                                                                                                                                                                                                                                                                                                                                                                                                                                                                                                                                                                                                                                            |                  |    |
|     | Uranium                                                                                                                                                                                                                                                                                                                                                                                                                                                                                                                                                                                                                                                                                                                                                       | = 3.8 -26.3      | 20 |
|     | or Tungsten                                                                                                                                                                                                                                                                                                                                                                                                                                                                                                                                                                                                                                                                                                                                                   |                  |    |
|     | or                                                                                                                                                                                                                                                                                                                                                                                                                                                                                                                                                                                                                                                                                                                                                            |                  |    |
|     | Niobium                                                                                                                                                                                                                                                                                                                                                                                                                                                                                                                                                                                                                                                                                                                                                       | = .9 - 6.7       |    |
|     | or                                                                                                                                                                                                                                                                                                                                                                                                                                                                                                                                                                                                                                                                                                                                                            |                  |    |
|     | Cerium                                                                                                                                                                                                                                                                                                                                                                                                                                                                                                                                                                                                                                                                                                                                                        | = .7 - 4.25      | 25 |
|     | or Boron                                                                                                                                                                                                                                                                                                                                                                                                                                                                                                                                                                                                                                                                                                                                                      |                  |    |
|     | Balance iron and negligible quantities of usual impurities.                                                                                                                                                                                                                                                                                                                                                                                                                                                                                                                                                                                                                                                                                                   |                  |    |
| (6) | Carbon                                                                                                                                                                                                                                                                                                                                                                                                                                                                                                                                                                                                                                                                                                                                                        | = less than .1   | 30 |
|     | Manganese                                                                                                                                                                                                                                                                                                                                                                                                                                                                                                                                                                                                                                                                                                                                                     | = .4 - .6        |    |
|     | Silicon                                                                                                                                                                                                                                                                                                                                                                                                                                                                                                                                                                                                                                                                                                                                                       | = less than .5   |    |
|     | Chromium                                                                                                                                                                                                                                                                                                                                                                                                                                                                                                                                                                                                                                                                                                                                                      | = 16 -18         |    |
|     | Molybdenum                                                                                                                                                                                                                                                                                                                                                                                                                                                                                                                                                                                                                                                                                                                                                    | = 1.8 - 2.4      |    |
|     | Tantalum                                                                                                                                                                                                                                                                                                                                                                                                                                                                                                                                                                                                                                                                                                                                                      | = 3 - 4.6        | 35 |
|     | or Niobium                                                                                                                                                                                                                                                                                                                                                                                                                                                                                                                                                                                                                                                                                                                                                    | = 1.5 - 2.3      |    |
|     | Balance iron and negligible quantities of usual impurities.                                                                                                                                                                                                                                                                                                                                                                                                                                                                                                                                                                                                                                                                                                   |                  |    |
| (7) | Carbon                                                                                                                                                                                                                                                                                                                                                                                                                                                                                                                                                                                                                                                                                                                                                        | = .2 - .3        | 40 |
|     | Manganese                                                                                                                                                                                                                                                                                                                                                                                                                                                                                                                                                                                                                                                                                                                                                     | = .4 - .6        |    |
|     | Silicon                                                                                                                                                                                                                                                                                                                                                                                                                                                                                                                                                                                                                                                                                                                                                       | = less than .5   |    |
|     | Chromium                                                                                                                                                                                                                                                                                                                                                                                                                                                                                                                                                                                                                                                                                                                                                      | = 23 -25         |    |
|     | Molybdenum                                                                                                                                                                                                                                                                                                                                                                                                                                                                                                                                                                                                                                                                                                                                                    | = 2.8 - 3.3      |    |
|     | Cerium                                                                                                                                                                                                                                                                                                                                                                                                                                                                                                                                                                                                                                                                                                                                                        | = 2.6 - 3.5      | 45 |
|     | or Zirconium                                                                                                                                                                                                                                                                                                                                                                                                                                                                                                                                                                                                                                                                                                                                                  | = 1.8 - 2.4      |    |
|     | Balance iron and negligible quantities of usual impurities.                                                                                                                                                                                                                                                                                                                                                                                                                                                                                                                                                                                                                                                                                                   |                  |    |
| (8) | Carbon                                                                                                                                                                                                                                                                                                                                                                                                                                                                                                                                                                                                                                                                                                                                                        | = .18- .22       | 50 |
|     | Manganese                                                                                                                                                                                                                                                                                                                                                                                                                                                                                                                                                                                                                                                                                                                                                     | = .4 - .6        |    |
|     | Silicon                                                                                                                                                                                                                                                                                                                                                                                                                                                                                                                                                                                                                                                                                                                                                       | = less than .5   |    |
|     | Chromium                                                                                                                                                                                                                                                                                                                                                                                                                                                                                                                                                                                                                                                                                                                                                      | = 27 -29         |    |
|     | Molybdenum                                                                                                                                                                                                                                                                                                                                                                                                                                                                                                                                                                                                                                                                                                                                                    | = 1.6 - 2        |    |
|     | Uranium                                                                                                                                                                                                                                                                                                                                                                                                                                                                                                                                                                                                                                                                                                                                                       | = 9 -12          | 55 |
|     | or Tungsten                                                                                                                                                                                                                                                                                                                                                                                                                                                                                                                                                                                                                                                                                                                                                   |                  |    |
|     | Balance iron and negligible quantities of usual impurities.                                                                                                                                                                                                                                                                                                                                                                                                                                                                                                                                                                                                                                                                                                   |                  |    |
|     | Titanium has heretofore been used in steels but primarily for the purpose of effecting de-oxidation thereof. This use is in no way comparable to our use of titanium. On the contrary, the presence of titanium in our steels serves the purposes of augmenting the corrosion resistance of the steel imparted by the molybdenum and of preventing the molybdenum from destroying the desired mechanical properties of the steel such as its cold rollability, cold ductility and cold malleability. Thus, the steels have a much greater resistance to corrosion than could be imparted to them by molybdenum alone, and at the same time are capable of being mechanically worked in the cold despite the presence of substantial quantities of molybdenum. | 60               |    |
|     |                                                                                                                                                                                                                                                                                                                                                                                                                                                                                                                                                                                                                                                                                                                                                               |                  | 65 |
|     |                                                                                                                                                                                                                                                                                                                                                                                                                                                                                                                                                                                                                                                                                                                                                               |                  | 70 |
|     |                                                                                                                                                                                                                                                                                                                                                                                                                                                                                                                                                                                                                                                                                                                                                               |                  | 75 |

The twofold function of the titanium in our steels is developed in the accompanying tables which compare the corrosion resistance and cold malleability of chromium-molybdenum steels with chromium-molybdenum-titanium steels. less than about .5% of silicon, from about 12 to about 30% of chromium, from about 1.5 to about 5% of molybdenum and a carbide-forming element of the 4th to 6th group of the Periodic System selected from the class consisting of 5

| 10 | C %                  | Mn %                                | Si %                       | Cr %                    | Mo %              | Ti %         | Loss of weight in grams/sq. meter of surface in 1 hour |                                                         |                                                                               |                                                            | 10 |
|----|----------------------|-------------------------------------|----------------------------|-------------------------|-------------------|--------------|--------------------------------------------------------|---------------------------------------------------------|-------------------------------------------------------------------------------|------------------------------------------------------------|----|
|    |                      |                                     |                            |                         |                   |              | Acetic acid conc. +5 gr. NaCl, temperature 90° C.      | 10% H <sub>2</sub> SO <sub>4</sub> , temperature 90° C. | 20% H <sub>2</sub> SO <sub>4</sub> + 4% HNO <sub>3</sub> , temperature 90° C. | Depth in mm. in a foil 1 mm. in thickness acc. to Erichsen |    |
| 15 | 0.10<br>0.08<br>0.07 | 0.40-0.60<br>0.40-0.60<br>0.40-0.60 | 0.30-1<br>0.30-1<br>0.30-1 | 14.92<br>15.97<br>17.60 | 2.0<br>2.0<br>2.0 | 0.45<br>0.93 | (*)<br>2.31<br>0.62                                    | 10.5<br>1.265<br>1.152                                  | 2.3<br>0.001<br>0.000                                                         | 7.3<br>10.85<br>10.40                                      | 15 |

  

| 20 | C %                                  | Mn %                                                          | Si %                                           | Cr %                                      | Mo %                                | Ti %                                    | Loss of weight in grams/sq. meter of surface in 1 hour |                                                                    |                                                                                                    |                                                            | 20 |
|----|--------------------------------------|---------------------------------------------------------------|------------------------------------------------|-------------------------------------------|-------------------------------------|-----------------------------------------|--------------------------------------------------------|--------------------------------------------------------------------|----------------------------------------------------------------------------------------------------|------------------------------------------------------------|----|
|    |                                      |                                                               |                                                |                                           |                                     |                                         | 10% H <sub>2</sub> SO <sub>4</sub> at 20° C.           | 20% H <sub>2</sub> SO <sub>4</sub> + 4% HNO <sub>3</sub> at 20° C. | NaOCl-solution containing 90 gms. of chlorine per lt. and 400 grams of CaCl <sub>2</sub> at 20° C. | Depth in mm. in a foil 1 mm. in thickness acc. to Erichsen |    |
| 25 | 0.27<br>0.07<br>0.20<br>0.08<br>0.27 | 0.40-0.60<br>0.40-0.60<br>0.40-0.60<br>0.40-0.60<br>0.40-0.60 | 0.30-1<br>0.30-1<br>0.30-1<br>0.30-1<br>0.30-1 | 24.83<br>26.70<br>26.28<br>29.15<br>26.28 | 2.0<br>2.30<br>1.88<br>1.71<br>4.00 | -----<br>-----<br>1.39<br>1.29<br>----- | 10.5<br>10.0<br>0.00<br>0.00<br>4.5                    | 0.027<br>(*)<br>0.0058<br>0.0000<br>(*)                            | Strong pitting<br>do<br>No attack<br>do<br>Pitting                                                 | 6.5<br>7.1<br>7.5<br>8.2<br>Not cold workable.             | 23 |
|    |                                      |                                                               |                                                |                                           |                                     |                                         |                                                        |                                                                    |                                                                                                    |                                                            |    |
| 30 | 0.27                                 | 0.40-0.60                                                     | 0.30-1                                         | 26.28                                     | 4.00                                | -----                                   |                                                        |                                                                    |                                                                                                    |                                                            | 30 |
|    |                                      |                                                               |                                                |                                           |                                     |                                         |                                                        |                                                                    |                                                                                                    |                                                            |    |

The asterisks in the above tables indicate that the results were not ascertained with particularity since it was apparent from observation that the test pieces had suffered a very material decrease in weight, a fact which was to be expected at the outset.

For a full discussion of the Erichsen test referred to in the tables attention is directed to page 154 of "Enzyklopädie der technischen Chemie" by Ullmann, volume 4, 2nd edition.

It is to be understood that similar results will be obtained when there is used, in place of titanium, the carbide forming elements mentioned above.

What we claim is:

Cold ductile and cold malleable corrosion-resistant alloys for use in the manufacture of articles which require resistance to attack by aqueous solutions of chlorine, calcium hypochlorite and their salts, containing less than .5% of carbon, from about .3 to about .6% of manganese,

tantalum, uranium, niobium, cerium, zirconium and tungsten, the zirconium being present in an amount of from about .5 to 3.5% while always exceeding by 6 to 12 times the amount of carbon, the tantalum being present in an amount of about 1.9 to 13.3% while always exceeding by about 23 to 46 times the amount of carbon, the uranium and tungsten being present in an amount of from about 3.8 to about 6.3% while always exceeding by about 45 to 90 times the amount of carbon, the niobium being present in an amount of from about .9 to about 6.7% while always exceeding by about 12 to 24 times the amount of carbon, and the cerium being present in an amount of about .7 to about 5% while always exceeding by about 9 to 18 times the amount of carbon, the balance being iron with the usual impurities.

HEINRICH REITZ.  
ERICH HENGLER.  
ALFRED BÜTTINGHAUS.

35

40

45

50